

# UNITED STATES PATENT OFFICE.

HENRY C. BAINES, OF EAST CLEVELAND, OHIO, ASSIGNOR, BY MESNE ASSIGNMENTS, TO THE CLEVELAND METAL PRODUCTS COMPANY, OF CLEVELAND, OHIO, A CORPORATION OF OHIO.

## TREATMENT OF STEEL, IRON, AND SIMILAR ARTICLES.

1,344,372.

Specification of Letters Patent. Patented June 22, 1920.

No Drawing.

Application filed September 6, 1916. Serial No. 118,745.

*To all whom it may concern:*

Be it known that I, HENRY C. BAINES, a subject of the King of Great Britain, residing at East Cleveland, Ohio, have invented 5 certain new and useful Improvements in the Treatment of Steel, Iron, and Similar Articles, of which the following is a specification.

This invention relates to the treatment 10 of iron or steel or articles having surfaces of iron or steel.

One object of the present invention is to provide iron or steel or articles having a surface of iron or steel with a protective 15 coating adapted to render the articles capable of resisting the action of moisture or other oxidizing or rusting influences. Another object of the invention is to prevent the solution from oxidizing, whereby the 20 articles to be treated may be effectively coated and the solution be maintained in efficient working condition. This results in coating the articles in a rapid and efficient manner and in a material saving of the solution 25 and of the ingredients contained therewithin. This object is realized by including in the solution an agent capable of evolving nascent hydrogen energetically, the hydrogen thus liberated combining with 30 any free oxygen in the solution to prevent the oxidation of the latter and maintain it in a working condition.

In carrying out the method of treating the articles, the latter are immersed in a solution 35 of a salt of phosphorous or hypophosphorous acid, or a mixture of the same, said solution being heated preferably to the boiling point. Through this treatment, the articles will be provided with a phosphite 40 or hypophosphite coating, intermingled with the original salt or salts, the articles being both impregnated and coated.

The nascent hydrogen may be evolved 45 from the surface of the articles by any of the usual methods. For instance, the articles may be made a cathode or cathodes of an electric circuit, or an alternating current may be used, or a dilute acid, such as sulfuric acid may be added as the agent to 50 set up the nascent hydrogen.

When the sulfuric or equivalent acid is added, phosphorous or hypophosphorous acid will be formed and hydrogen will be evolved in the body of the solution which

hydrogen, being in a nascent condition, will 55 exercise a reducing action upon the solution to prevent oxidation thereof.

A solution or compound which gives satisfactory results is as follows:

|                                  |           |    |
|----------------------------------|-----------|----|
| Ferrous phosphite $Fe_3(PO_3)_2$ | 1 lb.     | 60 |
| Water                            | 1 gallon. |    |
| Sulfuric acid                    | 2 ozs.    |    |

The proportions given are varied according to the nature of the iron or steel or 65 other metal to be treated and according to the nature of the coating desired. I may substitute zinc, cobalt, nickel, cadmium, chromium, or other phosphites or hypophosphites or mixtures of phosphites and 70 hypophosphites for a ferrous phosphite. For the sulfuric acid I may substitute hydrochloric or any other suitable acid of the proper strength.

For varying the texture or color of the 75 protective coating I may add substances of a gelatinous or amorphous nature, such for instance, as aluminum phosphate. For coloring or altering the texture of the coating I may add inert materials to the solution, 80 such for instance, as cobalt silicate or other inert silicates, oxids, etc. In the use of these agents for coloring or altering the texture of the coating it will be understood that the metal is immersed in a solution 85 of a salt or salts of phosphorous or hypophosphorous acids, or any combination thereof, and that by the added mixture of sulfuric acid with the solution, nascent-hydrogen will be evolved energetically therein or by the use of an electric current, such hydrogen will be evolved energetically at the surface of the articles, the nascent hydrogen combining with any free oxygen 90 that may be in the solution to prevent the 95 oxidation of the latter.

What is claimed, is:

1. The treatment of iron, steel, or articles having a surface of iron or steel, which comprises subjecting the same to the action 100 of a phosphite solution in the presence of an agent capable of preventing the oxidation of the solution.

2. The treatment of iron, steel, or articles having a surface of iron or steel, which 105 comprises subjecting the same to the action of a phosphite solution in the presence of nascent hydrogen.

3. The treatment of iron, steel, or articles having a surface of iron or steel, which comprises subjecting the same to the action of a solution of a phosphorous compound
- 5 capable of depositing with or forming upon said articles a protective coating in the presence of an agent capable of evolving nascent hydrogen in the body of said solution.
- 10 4. The treatment of iron, steel, or articles having a surface of iron or steel, which comprises subjecting the same to the action of a solution containing phosphorous acid in the presence of nascent hydrogen.
- 15 5. The treatment of iron, steel, or articles having a surface of iron or steel, which comprises subjecting the same to the action of a solution containing phosphorous and hypophosphorous acids in the presence of
- 20 nascent hydrogen.
6. The treatment of iron, steel, or articles having a surface of iron or steel, which comprises subjecting the same to the action of a solution containing phosphorous acid.
- 25 7. The treatment of iron, steel, or articles having a surface of iron or steel, which comprises subjecting the articles to the action of a solution containing a phosphorous salt in the presence of an acid capable of forming phosphorous acid with such salt.
- 30
8. The treatment of iron, steel, or articles having a surface of iron or steel, which comprises subjecting the articles to the action of a solution containing salts of phosphorous and hypophosphorous acids in the presence of sulfuric acid.
9. The treatment of iron, steel, or articles having a surface of iron or steel, which comprises subjecting the articles to the action of a solution containing ferrous phosphite, water and sulfuric acid in about the proportions specified.
10. A solution or compound for preventing the oxidation or rusting of iron or steel comprising ferrous phosphite, water, and an acid capable of forming phosphorous acid with such ferrous phosphite.
11. A solution or compound for preventing the oxidation or rusting of iron or steel comprising ferrous phosphite, water, and an acid capable of forming phosphorous acid with the ferrous phosphite and of evolving nascent hydrogen in such solution.
- In testimony whereof I affix my signature in the presence of two witnesses.

HENRY C. BAINES.

Witnesses:

R. BAINES,  
GEORGE A. HUBBARD.